

## 1

3,036,940

## EXPLOSIVE COMPOSITION

David A. Fletcher, Redlands, Calif., assignor to Lockheed Propulsion Company, a corporation of California  
No Drawing. Filed Jan. 21, 1958, Ser. No. 710,380  
2 Claims. (Cl. 149—78)

This invention relates to improvements in new and useful compositions of matter of the liquid or gel type suitable for use as explosives and fuels for rocket motors.

Explosives differ from ordinary combustibles in that they contain both oxidizing and reducing features and require no air or other supporter of combustion in order to react. These features may be both contained in the same molecular structure, such as nitroglycerin or nitrocellulose, or they may be combined as a heterogeneous, multiphase system such as sulfur-potassium nitrate-charcoal, i.e., gunpowder.

In all instances, shipment and handling has been a problem, as the prepared explosive is usually processed and packaged prior to use, after which it must be shipped to the location where it is to be used. Shipment and handling are extremely hazardous.

Most liquid propellants are of the bi-propellant type which consists of two strongly interacting liquids, one an oxidizer and the other a reducing agent. These, when combined under the proper conditions and ignited, burn rapidly with the liberation of much energy and gaseous products. Examples of such pairs are liquid oxygen/gasoline, or red fuming nitric acid/dimethyl hydrazine. These liquids have the disadvantages of requiring separate storage tanks and needing complicated feed mechanisms, pumps, turbines, or pressurizing devices, and a complicated thrust chamber. In the case of liquid oxygen, it cannot be stored for any extended period, because of its low critical pressure.

Another type of liquid propellant, used to a very limited extent commercially, are the monopropellants, which are complete rocket fuels in themselves and which contain both the oxidizing and reducing features. The present invention is of this type. Examples are hydrogen peroxide, nitromethane, ethylene oxide, tetranitromethane, or solutions of an organic material such as ethyl alcohol in hydrogen peroxide or tetranitromethane. They generally have the disadvantages of (1) low energy output, e.g., hydrogen peroxide, ethylene oxide; (2) poor storage stability; or (3) sensitivity to detonation, e.g., tetranitromethane; or they may have all three disadvantages. Concentrated hydrogen peroxide, 70-95% pure, has been used to some extent to provide auxiliary power for helicopters, but it has comparatively low energy, and trace impurities or contamination may cause spontaneous detonation. Nitromethane, while stable to ambient temperature storage, is low in energy and underoxidized to the point that carbon smoke may appear in the exhaust gas. Tetranitromethane, although capable of furnishing high impulse has thus far been too sensitive to detonation to be used to any extent as a monopropellant. Feed systems for monopropellants are comparatively simple since only one material is supplied to the rocket engine.

I have discovered that explosives and monopropellants may be prepared from safe, easily handled nonexplosive constituents which may be shipped with safety to the location of use, stored indefinitely and combined in solution when use is desired. Specifically, my invention contemplates lithium perchlorate in a solvent solution, preferably, low molecular weight polar organic solvents. Such solutions, once prepared, may be readily detonated.

Unlike other solid perchlorates, such as ammonium perchlorate, potassium perchlorate and sodium perchlorate which are soluble in organic solvents to a very limited ex-

## 2

tent, lithium perchlorate is unusually soluble, as the following table will reflect:

| 5  | Solvent       | Grams dissolved in 100 g. solvent |                   |                                  |                    |
|----|---------------|-----------------------------------|-------------------|----------------------------------|--------------------|
|    |               | LiClO <sub>4</sub>                | KClO <sub>4</sub> | NH <sub>4</sub> ClO <sub>4</sub> | NaClO <sub>4</sub> |
| 10 | Methanol      | 182.3                             | 0.11              | ( <sup>1</sup> )                 | 51.4               |
|    | Ethanol       | 151.8                             | 0.01              | ( <sup>1</sup> )                 | 14.7               |
|    | n-Propanol    | 105.0                             | 0.01              | ( <sup>1</sup> )                 | 4.0                |
|    | n-Butanol     | 79.3                              | 0.005             | ( <sup>1</sup> )                 | 1.9                |
|    | Acetone       | 156.3                             | 0.16              | ( <sup>1</sup> )                 | 51.7               |
|    | Diethyl ether | 113.7                             | insol.            | ( <sup>1</sup> )                 | insol.             |

<sup>1</sup> Solubility about like KClO<sub>4</sub>.

15 Any combination of the above solvents or other active solvents or diluents such as low molecular weight aliphatic nitro compounds, for example, nitromethane, nitroethane and dimethyl formamide, which exert solvent action on lithium perchlorate may be employed. The choice of solvent or solvents may be governed by the particular usage or the desired degree of vigor of reaction.

20 The following specific examples are illustrative of compositions contemplated by the present invention but in no manner limit the scope of the invention:

| 25                               | Percent by wt. |
|----------------------------------|----------------|
| (1) Anhydrous LiClO <sub>4</sub> | 62             |
| Methanol                         | 38             |
| (2) Anhydrous LiClO <sub>4</sub> | 15             |
| Nitromethane                     | 70             |
| Methanol                         | 15             |
| (3) Anhydrous LiClO <sub>4</sub> | 35             |
| Nitromethane                     | 35             |
| Methanol                         | 25             |
| Acetone                          | 5              |

35 Any suitable stabilizers, combustion catalysts or modifiers may be added as desired.

Compositions of the present invention, lithium perchlorate-methanol solution, for example, when employed as monopropellants, provide higher energy than any other monopropellant generally known in the art at the present time as shown by the following comparative data:

| 45                                                            | Propellant System | Density, lbs./in. <sup>3</sup> | I <sub>sp</sub> 1,000 | Volume Impulse                                                              | Remarks on Stability or Performance |
|---------------------------------------------------------------|-------------------|--------------------------------|-----------------------|-----------------------------------------------------------------------------|-------------------------------------|
| Hydrogen peroxide (90%).                                      | 0.050             | 150 max. low.                  | 7.5                   | Unstable, low impulse.                                                      |                                     |
| Nitromethane                                                  | 0.0412            | 173-----                       | 7.1                   | Detonates easily, smoky exhaust.                                            |                                     |
| Ethylene oxide                                                | 0.032             | 180-----                       | 5.8                   | Stable but low vol. impulse.                                                |                                     |
| 50 LiClO <sub>4</sub> -methanol solution (62% concentration). | 0.0497            | 226-----                       | 11.2                  | Stability of solute and solvent excellent; exhaust non-smoky, good impulse. |                                     |

55 Specific impulse, I<sub>sp</sub>, as used in the above table, is a parameter used in rocketry for rating energies of propellants and is the pounds thrust obtainable per pound-per-second or propellant flow under a given set of conditions.

60 Volume impulse, which is the product of specific impulse and density, gives a rating of propellants per unit of volume. Note that ethylene oxide has a moderately good specific impulse, but a low volume impulse due to its low density.

65 Monopropellant compositions preferably should contain a nitroparaffin such as nitromethane which improves fluidity yet allows the least reduction in specific impulse. The solubility of lithium perchlorate in methanol changes considerably with temperature and precipitation or gel formation may occur if nitromethane or other diluent is not added.

## I claim:

1. A liquid monopropellant composition which consists essentially of about 62% by weight of lithium perchlorate in solution with about 38% of methanol.

2. A liquid monopropellant composition which consists essentially of about 15-35% by weight of lithium perchlorate in solution with about 35-70% of a lower nitro-paraffin and about 15-25% by weight of methanol.

## References Cited in the file of this patent

## UNITED STATES PATENTS

2,783,138 Parsons ----- Feb. 26, 1957

## OTHER REFERENCES

- Leonard: "Journal of the American Rocket Society," No. 72, December 1947, pages 10-16.
- "Jet Propulsion," Report prepared by the Guggenheim Aeronautical Laboratory and the Jet Propulsion Laboratory, GALCIT, California Institute of Technology for the Air Technical Service Command, 1946, pages 295-296.
- Lange's Handbook of Chemistry, 7th ed., Handbook Publishers, Inc., Sandusky, Ohio, 1949, pp. 228-229.
- 10 Tschinkel: Ind. and Eng. Chemistry, vol. 48, No. 4, pp. 732-735, April 1956.